

## 1

3,130,117

INCREASING THE STRENGTH OF PAPER WITH  
VINYL SULFONIUM POLYMERS

Charles G. Humiston, Frederick J. Meyer, and Duane L. Kenaga, all of Midland, Mich., assignors to The Dow Chemical Company, Midland, Mich., a corporation of Delaware  
No Drawing. Filed Mar. 13, 1961, Ser. No. 95,015  
7 Claims. (Cl. 162—168)

This invention relates to the use of water-soluble homopolymers and copolymers of certain vinyl sulfonium compounds as beater additives to improve the physical properties of cellulosic and lignocellulosic articles such as paper, hardboard and insulation board.

In the making of paper, hardboard, insulation board and the like various non-fibrous materials may be added to the stock at or beyond the beater prior to article formation. Such materials are known as beater additives and are employed to improve the properties of the finished product such as dry and wet strength, water repellancy, dimensional stability, rot and mildew resistance and rodent repellancy. Certain additives may increase machine speed, reduce loss of fines, reduce refining costs, permit the use of a larger percentage of inert fillers, or allow an increase in the use of less expensive short fibered pulp.

Beater additives may be added at the beater, or at other points in the process up to and including the head box. In certain machines it is possible to introduce the beater additives at other points between the refiner and the head box, such as the machine chest, stuff box, fan pump or Jordan box.

Strong cellulosic articles are obtained through the use of long-fibered woods in the preparation of the pulp. However, the supply of soft woods which are long fibered is insufficient to meet the growth demands of the pulp and paper industry and the use of hardwoods, which are short fibered, is increasing. It is, therefore, a desideratum of the art, to provide additives which will increase both the dry and wet strength of articles manufactured from cellulosic and lignocellulosic materials.

We have now found that such articles may be obtained by adding from about 0.025 to 5.0, preferably from about 0.1 to 3.0 weight percent, dry fiber basis, of one or more water-soluble homopolymers and copolymers of vinyl sulfonium compounds to the fiber slurry at or beyond the beater prior to article formation. The homopolymers used in the present invention may be represented by the general formula



wherein R<sub>1</sub> is selected from the group consisting of hydrogen and alkyl radicals containing from 1 to 6 carbon

## 2

atoms, X is an organic sulfur-containing radical selected from the group consisting of (A) sulfides of the formula, R<sub>2</sub>SR<sub>3</sub>, wherein R<sub>2</sub> and R<sub>3</sub> each represents a member of the group consisting of (1) alkyl radicals containing from 1 to 6 carbon atoms, (2) haloalkyl radicals containing from 1 to 6 carbon atoms, (3) hydroxyalkyl radicals containing from 1 to 6 carbon atoms; (4)



10 wherein n is an integer from 1 to 4 inclusive; (5)



15 wherein n is an integer from 1 to 4 inclusive; (6)



wherein m is an integer from 1 to 5; (7) —C<sub>n</sub>H<sub>2n</sub>COOH; (8) —C<sub>n</sub>H<sub>2n</sub>COOC<sub>n</sub>H<sub>2n+1</sub>; (9) —C<sub>n</sub>H<sub>2n</sub>COO alkali metal; and (10) —C<sub>n</sub>H<sub>2n</sub>CONH<sub>2</sub>; wherein n in substituents (7), (8), (9) and (10) is an integer from 1 to 5

20 with the total number of carbon atoms in each of the substituents (7), (8), (9), and (10) not exceeding 6, and where the total number of carbon atoms of the R<sub>2</sub> and R<sub>3</sub> groups attached to a common sulfur atom does not exceed 18 and (B) cyclic thio compounds selected from the group consisting of tetrahydrothiophene, hydroxy substituted tetrahydrothiophene, halo substituted tetrahydrothiophene, alkyl substituted tetrahydrothiophene where alkyl refers to groups containing from 1 to 5 carbon atoms, tetrahydrothiopyran, and 1,4-oxathiane; 25 and Y is an anion such as carbonate, oxalate, phthalate, succinate, dihydrogen phosphate, fluoride, benzoate, chloride, nitrate, acetate, sulfate, bromide, iodide and the like.

30 The monomers useful in preparing the polymers to be used in this invention are made by contacting a vinylbenzyl halide with an organic sulfur containing compound in the presence or absence of a solvent or non-solvent liquid medium. The polymers may be produced by subjecting the monomers to the polymerization methods conventionally used with free radical catalyzed aqueous systems, i.e., emulsion-, and solution polymerization in the presence of actinic light, ultra-violet irradiation, gamma radiation, "azo" catalysts and peroxides.

35 In preparing the monomers of this invention, a vinylbenzyl halide such as the chloride, bromide, or iodide is reacted with an organic sulfur-containing compound as defined heretofore. Theoretical molar equivalents of the vinylbenzyl halide and the sulfur-containing compound 40 ordinarily are used, although from 50 percent up to 200 percent stoichiometric amounts of the organic sulfur-containing compounds can be used. An excess of about 200 percent of the stoichiometric value in some cases 45 promotes the formation of the vinylbenzyl sulfonium halide monomer. This excess of the sulfur containing reactant is recoverable from the reaction mixture. If the reactants are liquid, preparation of the monomer can be carried out without use of a solvent, but solvents such as water, nitromethane, methanol, ethanol, acetonitrile and the like can be used. The reaction can be carried

out at temperatures from about room temperature up to about 100° C.; but reaction temperatures from about 30° to about 80° C. are preferred. The reaction normally will be carried out at substantially atmospheric pressure, but superatmospheric pressure sufficient to prevent loss of volatile reactants can be employed. A minimum reaction time of about 2 to about 4 hours results in formation of certain of the monomeric sulfonium compounds. However, this reaction time will vary with the different molecular species and reaction times of 24 hours or more can be employed.

The vinylbenzyl sulfonium monomers, as produced, will have a halide anion. If desired this halide form of the monomer can be converted in a conventional manner to any one of a number of common anionic forms such as carbonate, nitrate, sulfate, acetate and the like by passing a solution of the monomer into contact with an anion exchange resin in the proper salt form.

Preparation of the homopolymers and/or copolymers is conveniently carried out by polymerizing the monomeric sulfonium compound with or without another polymerizable monomer such as acrylamide, polyolefins, acrylic acid, vinylaromatic monomers, acrylates and methacrylates, acrylonitrile, trimethyl(ar-vinylbenzyl) ammonium chloride, and the like in an emulsion or solution in the presence of vinyl polymerization catalyst such as ultraviolet light, gamma radiation, "azo" catalysts, peroxides, and the like for a period of time ranging from 4 hours to two weeks or more.

In some instances the polymeric products useful in the present invention may be prepared by other routes such as by introducing a halomethyl group into an aromatic polymer substrate and thereafter reacting with a thioether. Because of the difficulty in obtaining a uniform distribution of the introduced halomethyl groups and the difficulty of obtaining an effective reaction of such products with the thioether, this route is not generally desirable.

The homopolymers and copolymers may be lightly cross-linked with any of the conventional cross-linking agents such as divinylbenzene (DVB), the divinyl ether of diethylene glycol, ethylene glycol diacrylate, ethylene glycol, diacrylate, ethylene glycol dimethacrylate, glycerol trimethacrylate, dialkyl itaconate, diallyl, maleate, diallyl fumarate, diisopropenyl diphenyl, the close homologues, equivalents, and the like of the foregoing, or mixtures thereof. When prepared in an emulsion and when in a swelling medium, the polymers are referred to herein as microgels. The polymers, especially the microgels often advantageously can be prepared by emulsion polymerization of the vinylbenzyl halide followed by reaction with the desired sulfur-containing compound, although this method is less effective in some cases than the above described procedure.

Polymers useful in the present invention include homopolymers of vinylbenzyl bis(2-hydroxyethyl)sulfonium chloride, vinylbenzyl methylthetin, vinylbenzyl-2-hydroxyethanolthetin, vinylbenzyl methyl(3-carboxy-3-hydroxypropyl)sulfonium hydroxide, inner salt; vinylbenzyl bis(2-carboxyethyl)sulfonium hydroxide, inner salt; vinylbenzyl methyl 2-hydroxyethyl sulfonium chloride and the like.

The molecular weight of the homopolymers and copolymers used in the present invention is not critical. It is necessary for the polymer to bear a multiplicity of positive charges so it will adsorb effectively on the paper pulp. Linear polymers having a molecular weight up to 100,000 or more and lightly cross-linked polymers and microgels having molecular weights from 100,000 up to 200, or more, million have been found to be equally effective in improving the wet and dry strength, water resistance, flexural strength, etc. of the finished cellulosic article.

As little as 0.025 weight percent, dry fiber basis, of the sulfonium homopolymers or copolymers will produce a

marked improvement in the physical properties of the resulting cellulosic article although from 0.1 to 3.0 weight percent is preferable. A greater amount may be used if desired, but is usually disadvantageous for economic considerations.

With the use of the additives of this invention it is possible to reduce the beating time and still maintain a desired level of dry bursting strength in the finished product. Alternatively, a higher level of dry bursting strength may be obtained than would be obtainable by using increased beating time alone. As increased beating does not increase wet strength, it is possible, with the use of the additives of this invention, to reduce beating time while maintaining a desired level of dry bursting strength and at the same time increasing wet strength with no decrease in the tearing resistance.

The pH of the pulp slurry to be treated is not critical, and may vary from acid to alkaline. A pH in the range of from about 4.0 to 10.0 is preferably used.

In order to attain maximum strength improvement with the sulfonium additives of this invention it is necessary to completely "cure" the resin in the product by heating and drying.

The additives of the present invention are equally effective when no alum is used as an inorganic flocculant and when up to 10 percent alum is added.

The present invention may be better understood by reference to the following examples which are not to be construed as limiting.

30

#### EXAMPLE I

Unbleached mixed hardwoods soda pulp was beaten in a Valley beater to a freeness of 360 ml. (Canadian standard freeness). Five grams of the beaten pulp were dispersed in approximately 2 liters of water. Various concentrations of three microgels were added to the pulp slurry from dilute solutions (0.1 to .5 percent in water). After stirring 3 minutes the slurry was diluted further with tap water and hand sheets made up. All sheets were dried for 30 minutes at 90-110° C. Bursting strength was determined according to standard TAPPI procedures. Results are as follows.

Table I

| Run | Additive                                                                | Weight Percent | pH of Pulp Slurry | Dry Bursting Strength |                             |
|-----|-------------------------------------------------------------------------|----------------|-------------------|-----------------------|-----------------------------|
|     |                                                                         |                |                   | Burst Factor, p.s.i.  | Percent Change from Control |
| 50  | None (Control)                                                          |                |                   | 28.9                  |                             |
| 50  | Poly(dimethyl ar-vinylbenzyl sulfonium chloride), 0.04% divinylbenzene. | 0.1            | 5.1               | 31.9                  | +10.4                       |
| 55  | do                                                                      | 0.5            | 5.1               | 40.1                  | +38.8                       |
| 55  | do                                                                      | 1.0            | 5.1               | 46.5                  | +60.9                       |
| 55  | do                                                                      |                | 4.9               | 42.3                  | +46.4                       |
| 60  | Above sulfonium-containing no divinylbenzene.                           | 1.0            | 5.0               | 44.5                  | +54.0                       |
| 60  | Above sulfonium with 0.80% divinylbenzene.                              | 1.0            | 5.1               | 39.3                  | +36.0                       |

#### EXAMPLE II

The effect of beating time on unbleached soda pulp and cotton linters with and without the additives of the present invention is shown in Tables II and III. The sulfonium polymer is poly[ar-vinylbenzyl-bis(2-hydroxyethyl)sulfonium]chloride and is essentially linear. The microgel is poly(dimethyl[ar-vinylbenzyl]sulfonium chloride) which is crosslinked with 0.06 weight percent divinylbenzene. At each freeness aliquots of pulp slurry containing 5 grams of pulp were removed and tested. Handsheets were made up and wet and dry burst and dry tear were determined by standard test methods, i.e. TAPPI standard T220-m-53.

75

Table II

## EFFECT OF BEATING TIME USING UNBLEACHED SODA PULP

| Run | Treatment    | Beating Time (Min.) | Canadian Standard Freeness (Ml.) | Dry Burst Factor | Percent Increase in Burst over Control | Wet Burst Factor | Percent Wet Burst/Dry Control |
|-----|--------------|---------------------|----------------------------------|------------------|----------------------------------------|------------------|-------------------------------|
| 1   | Control      | 21                  | 552                              | 10.1             | 0                                      | 5.3              | 52.5                          |
| 2   | 1% sulfonium | 21                  | 552                              | 23.3             | 130.7                                  | 0                |                               |
| 3   | Control      | 32                  | 460                              | 18.3             | -----                                  | 9.5              | 51.9                          |
| 4   | 1% sulfonium | 32                  | 460                              | 34.5             | 88.5                                   | 0                |                               |
| 5   | Control      | 40                  | 396                              | 24.3             | -----                                  | 11.9             | 49.0                          |
| 6   | 1% sulfonium | 40                  | 396                              | 41.7             | 71.6                                   | 0                |                               |
| 7   | Control      | 50                  | 288                              | 31.4             | -----                                  | 0                |                               |
| 8   | 1% sulfonium | 50                  | 288                              | 48.2             | 53.5                                   | 15.1             | 48.1                          |
| 9   | Control      | 60                  | 186                              | 36.6             | -----                                  | 0                |                               |
| 10  | 1% sulfonium | 60                  | 186                              | 49.4             | 35.0                                   | 16.2             | 44.3                          |

Table III

## EFFECT OF BEATING TIME ON COTTON LINTERS

| Run | Treatment    | Beating Time (Min.) | Canadian Standard Freeness (Ml.) | Dry Burst Factor | Percent Increase in Burst over Control | Wet Burst Factor | Percent Wet Burst/Dry Control | Tear Factor |
|-----|--------------|---------------------|----------------------------------|------------------|----------------------------------------|------------------|-------------------------------|-------------|
| 1   | Control      | 19                  | 487                              | 6.9              | 0                                      | 7.1              | 73.9                          |             |
| 2   | 1% sulfonium | 19                  | 487                              | 14.9             | 159.4                                  | 6.7              | 97.1                          | 93.8        |
| 3   | Control      | 40                  | 306                              | 11.4             | -----                                  | 4.1              | 87.2                          |             |
| 4   | 1% sulfonium | 40                  | 306                              | 20.7             | 81.6                                   | 9.3              | 81.6                          | 98.0        |
| 5   | 1% microgel  | 40                  | 306                              | 18.4             | 61.4                                   | -----            | -----                         |             |
| 6   | Control      | 60                  | 168                              | 12.9             | 0                                      | 0                | 87.5                          |             |
| 7   | 1% sulfonium | 60                  | 168                              | 25.4             | 96.9                                   | 11.3             | 87.6                          | 95.4        |
| 8   | 1% microgel  | 60                  | 168                              | 19.9             | 54.3                                   | -----            | -----                         |             |
| 9   | Control      | 80                  | 76                               | 14.0             | -----                                  | 1.0              | 77.6                          |             |
| 10  | 1% sulfonium | 80                  | 76                               | 21.8             | 55.7                                   | 10.2             | 72.9                          | 84.7        |
| 11  | 1% microgel  | 80                  | 76                               | 23.0             | 64.3                                   | -----            | -----                         |             |

Tables IV through XI illustrate the effects of variables such as pH, concentration, molecular weight, type of pulp, addition of alum, and the use of various copolymers and homopolymers within the scope of this invention. For these experiments the pulp was prepared by adding 360 grams of air-dry pulp and 23 liters of water to a 1½ pound Valley laboratory beater and beating to a Canadian standard freeness of about 400 ml. Aliquots containing 5 grams of pulp were removed for each handsheet. Two liters of water were added to the aliquot, and the test material added with stirring. The dilute slurry was added to the sheet mold and the handsheets

45 prepared according to a modification of TAPPI standard T205-m-53. The sheets were oven dried, conditioned at least 48 hours at 21° C. and 62 percent relative humidity, and tested for dry burst, tensile and tear according to TAPPI standard T220-m-53. Wet bursting strength 50 was determined after soaking the test samples in deionized water for 4-24 hours. All tests were corrected for basis weight of the papers. Unless otherwise noted the pulp used was unbleached hardwood soda pulp. In each 55 case the percent additive is based on dry weight of the pulp.

Table IV

## EFFECT OF pH ON THE ACTIVITY OF POLY [α-VINYLBENZYL-BIS(2-HYDROXYETHYL) SULFONIUM CHLORIDE] (ESSENTIALLY LINEAR)

| Run | Treatment    | pH  | Dry Burst Factor | Percent Increase in Burst over Control | Wet Burst Factor | Percent Wet Burst/Dry Control | Breaking Length (Meters) | Percent Increase over Control | Tear Factor |
|-----|--------------|-----|------------------|----------------------------------------|------------------|-------------------------------|--------------------------|-------------------------------|-------------|
| 1   | Control      | 4.5 | 21.9             | 0                                      | 0                | 4,100                         | 88.1                     |                               |             |
| 2   | 1% sulfonium | 4.5 | 38.2             | 74.4                                   | 10.7             | 48.9                          | 5,530                    | 34.9                          | 90.0        |
| 3   | Control      | 7.0 | 22.5             | 0                                      | 0                | 4,230                         | 87.8                     |                               |             |
| 4   | 1% sulfonium | 7.0 | 38.6             | 71.6                                   | 11.1             | 49.3                          | 5,840                    | 38.1                          | 94.7        |
| 5   | Control      | 9.5 | 21.7             | 0                                      | 0                | 4,010                         | 89.7                     |                               |             |
| 6   | 1% sulfonium | 9.5 | 40.0             | 84.3                                   | 12.6             | 58.1                          | 5,660                    | 41.1                          | 94.9        |

7  
**Table V**  
 EFFECT OF CONCENTRATION

| Run | Treatment                                                                                | Concen-<br>tration<br>of<br>Additive<br>Weight<br>(percent) | Dry<br>Burst<br>Factor | Percent<br>Increase<br>in<br>Burst<br>over<br>Control | 5 Run | Furnish | Free-<br>ness | Additive | Percent<br>Increase<br>in Dry<br>Burst |
|-----|------------------------------------------------------------------------------------------|-------------------------------------------------------------|------------------------|-------------------------------------------------------|-------|---------|---------------|----------|----------------------------------------|
| 1   | Control                                                                                  | 0                                                           | 22.3                   |                                                       |       |         |               |          |                                        |
| 2   | Poly ar-vinylbenzyl-bis-(2-hydroxyethyl) sulfonium chloride (linear).                    | 0.5                                                         | 36.2                   | 62.3                                                  | 10    |         |               |          |                                        |
| 3   | do                                                                                       | 1.0                                                         | 40.0                   | 79.4                                                  |       |         |               |          |                                        |
| 4   | do                                                                                       | 1.5                                                         | 43.2                   | 93.7                                                  |       |         |               |          |                                        |
| 5   | do                                                                                       | 2.0                                                         | 41.3                   | 85.2                                                  |       |         |               |          |                                        |
| 6   | do                                                                                       | 2.5                                                         | 42.2                   | 89.2                                                  |       |         |               |          |                                        |
| 7   | do                                                                                       | 3.0                                                         | 41.9                   | 87.9                                                  | 15    |         |               |          |                                        |
| 8   | Control                                                                                  | 0                                                           | 28.9                   |                                                       |       |         |               |          |                                        |
| 9   | Poly(dimethyl[ar-vinyl-benzyl] sulfonium chloride) with 0.04% divinylbenzene (Microgel). | 0.1                                                         | 31.9                   | 10.4                                                  |       |         |               |          |                                        |
| 10  | do                                                                                       | 0.5                                                         | 40.1                   | 38.8                                                  |       |         |               |          |                                        |
| 11  | do                                                                                       | 1.0                                                         | 46.5                   | 60.9                                                  |       |         |               |          |                                        |
| 12  | do                                                                                       | 3.0                                                         | 42.3                   | 46.4                                                  | 20    |         |               |          |                                        |

8  
**Table VII**  
 EFFECT OF PULP FURNISH ON BURST

Table VI  
 EFFECT OF POLYMER SIZE OF POLY[DIMETHYL(ar-VINYLBENZYL)SULFONIUM CHLORIDE] MICROGELS 25

| Run | 1% sulfonium polymer <sup>1</sup>     | Approximate<br>Molecular<br>Weight | Burst<br>Factor | Percent<br>Increase<br>in Burst<br>over<br>Control | 30 |
|-----|---------------------------------------|------------------------------------|-----------------|----------------------------------------------------|----|
| 1   | Control                               |                                    | 21.3            |                                                    |    |
| 2   | 0.8% DVB <sup>2</sup>                 | 200 million                        | 32.2            | 51.2                                               |    |
| 3   | 0.4% DVB                              | do                                 | 37.3            | 75.1                                               |    |
| 4   | 0.2% DVB                              | do                                 | 34.9            | 63.8                                               |    |
| 5   | 0.08% DVB                             | do                                 | 40.2            | 88.7                                               |    |
| 6   | 0.06% DVB                             | do                                 | 38.0            | 78.4                                               | 35 |
| 7   | 0.05% DVB                             | do                                 | 38.0            | 78.4                                               | 1  |
| 8   | 0.04% DVB                             | do                                 | 34.9            | 63.8                                               | 2  |
| 9   | 0.02% DVB                             | do                                 | 36.3            | 70.4                                               | 3  |
| 10  | 0.00% DVB                             | 1.75 million                       | 37.0            | 73.7                                               | 4  |
| 11  | 0.00% DVB                             |                                    |                 |                                                    | 5  |
| 12  | 0.01% DDM <sup>2</sup>                | 1.36 million                       | 39.7            | 86.4                                               | 6  |
| 13  | 0.00% DVB 0.01% DDM <sup>3</sup>      | 450,000                            | 39.2            | 84.0                                               | 7  |
|     | Linear sulfonium polymer <sup>3</sup> | 100,000                            | 38.4            | 80.3                                               | 8  |

Table VIII  
 EFFECT OF ALUM ADDITION

| Run | Treatment                 | Weight<br>Percent<br>Alum<br>Added <sup>1</sup> | Dry<br>Burst<br>Factor | Percent<br>Increase<br>in Burst<br>over<br>Control | Wet<br>Burst<br>Factor |
|-----|---------------------------|-------------------------------------------------|------------------------|----------------------------------------------------|------------------------|
| 1   | Control                   | 0                                               | 23.0                   |                                                    | 0                      |
| 2   | 1% sulfonium <sup>2</sup> | 0                                               | 40.6                   | 76.5                                               | 11.9                   |
| 3   | Control                   | 1.0                                             | 23.9                   |                                                    | 0                      |
| 4   | 1% sulfonium              | 1.0                                             | 41.4                   | 73.2                                               | 12.3                   |
| 5   | Control                   | 3.0                                             | 24.3                   |                                                    | 1.3                    |
| 6   | 1% sulfonium              | 3.0                                             | 38.1                   | 56.8                                               | 11.0                   |
| 7   | Control                   | 5.0                                             | 22.3                   |                                                    | 1.3                    |
| 8   | 1% sulfonium              | 5.0                                             | 39.0                   | 74.9                                               | 12.7                   |
| 9   | Control                   | 10.0                                            | 23.6                   |                                                    | 1.1                    |
| 10  | 1% sulfonium              | 10.0                                            | 38.3                   | 62.3                                               | 12.1                   |

<sup>1</sup> Emulsion polymerization of vinylbenzyl chloride followed by reaction with dimethyl sulfide.

<sup>2</sup> DVB = divinylbenzene; DDM = dodecylmercaptan.

<sup>3</sup> Solution polymerization of sulfonium monomer.

<sup>1</sup> Based on the weight of dry fiber present.

<sup>2</sup> Sulfonium represents poly[ar-vinylbenzyl-bis(2-hydroxyethyl)sulfonium chloride].

Table IX

HANDSHEETS TREATED WITH COPOLYMERS OF DIMETHYL(ar-VINYLBENZYL)SULFONIUM CHLORIDE AND OTHER MONOMERS

| Run | Other Monomer      | Weight<br>percent<br>other<br>Mon-<br>omer in<br>copol-<br>ymer | Weight<br>Percent<br>of Copol-<br>ymer Em-<br>ployed | Dry<br>Burst<br>Factor | Percent<br>Increase<br>in Burst<br>over<br>Control | Wet<br>Burst<br>Factor | Tear<br>Factor |
|-----|--------------------|-----------------------------------------------------------------|------------------------------------------------------|------------------------|----------------------------------------------------|------------------------|----------------|
| 1   | Styrene            | 80                                                              | 1.0                                                  | 29.2                   | 32.1                                               | 3.3                    | 102.3          |
| 2   | do                 | 60                                                              | 1.0                                                  | 34.1                   | 54.3                                               | 9.5                    | 97.7           |
| 3   | do                 | 40                                                              | 1.0                                                  | 34.5                   | 56.1                                               | 9.1                    | 101.2          |
| 4   | do                 | 40                                                              | 0.67                                                 | 32.6                   | 23.0                                               | 6.9                    |                |
| 5   | Acrylonitrile      | 80                                                              | 1.0                                                  | 46.8                   | 46.8                                               | 10.0                   | 101.2          |
| 6   | do                 | 60                                                              | 1.0                                                  | 39.7                   | 68.9                                               | 11.3                   | 97.6           |
| 7   | do                 | 40                                                              | 1.0                                                  | 38.6                   | 64.3                                               | 10.9                   | 99.4           |
| 8   | do                 | 20                                                              | 1.0                                                  | 41.3                   | 75.7                                               | 11.6                   | 101.2          |
| 9   | do                 | 40                                                              | 0.5                                                  | 33.4                   | 26.0                                               | 6.5                    |                |
| 10  | Acrylic Acid       | 3                                                               | 1.0                                                  | 30.7                   | 75.7                                               | 11.4                   | 104.3          |
| 11  | Acrylamide         | 5                                                               | 1.0                                                  | 36.8                   | 62.8                                               | 10.5                   | 103.4          |
| 12  | Methylmethacrylate | 20                                                              | 1.0                                                  | 34.6                   | 47.2                                               | 7.8                    |                |

<sup>1</sup> (0.04-0.06 percent DVB.)

Table X

PROPERTIES OF HANDEETS TREATED WITH COPOLYMERS OF BIS(2-HYDROXYETHYL) ar-VINYLBENZYL SULFONIUM CHLORIDE AND OTHER MONOMERS

| Run | Copolymer     |              | Weight Percent | Dry Burst Factor | Percent Increase over Control | Wet Burst Factor | Tensile Breaking Length (Meters) | Percent Increase over Control |
|-----|---------------|--------------|----------------|------------------|-------------------------------|------------------|----------------------------------|-------------------------------|
|     | Other Monomer | Mole Percent |                |                  |                               |                  |                                  |                               |
| 1   | Ammonium a    | 50           | 1.0            | 30.8             | 25.7                          | 6.1              | 4,820                            | 25.2                          |
| 2   | do b          | 49           | 1.0            | 33.6             | 37.1                          | 8.1              | 4,940                            | 28.3                          |
| 3   | do a          | 65           | 0.5            | 36.8             | 59.3                          | 9.7              |                                  |                               |
| 4   | Sulfonium c   | 44           | 1.0            | 36.2             | 47.8                          | 10.1             | 5,410                            | 40.5                          |
| 5   | Acrylamide    | 40           | 0.5            | 35.6             | 49.0                          | 8.7              |                                  |                               |
| 6   | Acrylic Acid  | 50           | 0.5            | 41.1             | 77.9                          | 12.2             |                                  |                               |

a Ammonium=trimethyl (ar-vinylbenzyl) ammonium chloride.

b Microgel polymer containing 0.04-0.06 weight percent divinylbenzene (DVB).

c Sulfonium=dimethyl (ar-vinylbenzyl) sulfonium chloride.

Table XI

PROPERTIES OF HANDEETS TREATED WITH OTHER POLYMERS WITHIN THE SCOPE OF THIS INVENTION

| Run | Polymer                                                                                    | Weight Percent | Dry Burst Factor | Percent Increase over Control | Wet Burst Factor | Percent Wet Burst/Dry Control | Percent Wet Burst/Dry Burst |
|-----|--------------------------------------------------------------------------------------------|----------------|------------------|-------------------------------|------------------|-------------------------------|-----------------------------|
| 1   | Poly(vinylbenzyl)bis(2-hydroxyethyl)sulfonium chloride]                                    | 1.0            | 33.6             | 54.1                          | 6.5              | 29.8                          | 19.3                        |
| 2   | do                                                                                         | 1.0            | 31.5             | 44.5                          | 4.0              | 18.3                          | 12.7                        |
| 3   | Poly(vinylbenzyl)methyl-2,3-dihydroxypropylsulfonium chloride]                             | 1.0            | 37.3             | 9.4                           | 7.2              | 21.1                          | 19.3                        |
| 4   | Poly(vinylbenzyl)-2-hydroxyethyl-2-carbamoylethylsulfonium chloride]                       | 1.0            | 32.3             | 31.8                          | 5.6              | 22.9                          | 17.3                        |
| 5   | Poly(vinylbenzyl)methyl-2-carbamoylethylsulfonium chloride]                                | 1.0            | 31.1             | 26.9                          | 5.1              | 20.8                          | 16.4                        |
| 6   | Poly(vinylbenzyl)methyl-2-hydroxyethylsulfonium chloride]                                  | 1.0            | 32.8             | 33.9                          | 5.3              | 21.6                          | 16.2                        |
| 7   | Poly(vinylbenzyl)methyl(carbamoylmethyl)sulfonium chloride]                                | 1.0            | 33.9             | 38.4                          | 6.9              | 28.2                          | 20.4                        |
| 8   | Poly(vinylbenzyl)methyl thetin]                                                            | 1.0            | 28.3             | 6.4                           | 1.6              | 6.0                           | 5.7                         |
| 9   | Poly(vinylbenzyl)ethanol thetin+alum                                                       | 1.0            | 34.6             | 30.1                          | 7.9              | 29.7                          | 22.8                        |
| 10  | Poly(vinylbenzyl)methionium chloride]                                                      | 1.0            | 33.0             | 1.5                           | 10.5             | 31.3                          | 31.8                        |
| 11  | Poly(vinylbenzyl)-bis(2-hydroxyethyl)sulfonium bicarbonate]                                | 1.0            | 26.7             | 25.4                          | 2.3              | 10.0                          | 8.6                         |
| 12  | Poly(vinylbenzyl)-bis(2-hydroxyethyl)sulfonium acetate]                                    | 1.0            | 29.9             | 40.4                          | 3.3              | 14.3                          | 10.0                        |
| 13  | Poly(vinylbenzyl)-bis(2-hydroxyethyl)sulfonium dihydrogenphosphate]                        | 1.0            | 27.0             | 26.8                          | 4.1              | 17.8                          | 15.2                        |
| 14  | Poly(vinylbenzyl)-bis(2-hydroxyethyl)sulfonium sulfate]                                    | 1.0            | 28.1             | 31.9                          | 2.8              | 12.2                          | 10.0                        |
| 15  | Poly(vinylbenzyl)-bis(2-hydroxyethyl)sulfonium bromide]                                    | 1.0            | 26.9             | 26.3                          | 2.7              | 11.7                          | 10.0                        |
| 16  | Poly(vinylbenzyl)-bis(2-hydroxyethyl)sulfonium fluoride]                                   | 1.0            | 26.7             | 25.4                          | 2.4              | 10.4                          | 9.0                         |
| 17  | Poly(vinylbenzyl)-bis(2-hydroxyethyl)sulfonium nitrate]                                    | 1.0            | 27.2             | 27.7                          | 2.3              | 10.0                          | 8.5                         |
| 18  | Poly(vinylbenzyl)-bis(2-hydroxyethyl)sulfonium benzoate]                                   | 1.0            | 26.8             | 25.8                          | 2.5              | 10.9                          | 9.3                         |
| 19  | Poly(vinylbenzyl)-bis(2-hydroxyethyl)sulfonium phthalate]                                  | 1.0            | 29.4             | 38.0                          | 4.5              | 19.6                          | 15.3                        |
| 20  | Poly(vinylbenzyl)-bis(2-hydroxyethyl)sulfonium carbamate]                                  | 1.0            | 27.9             | 31.0                          | 3.4              | 14.8                          | 12.2                        |
| 21  | Poly(vinylbenzyl)-bis(2-hydroxyethyl)sulfonium succinate]                                  | 1.0            | 29.0             | 36.2                          | 4.3              | 18.7                          | 14.8                        |
| 22  | Poly(vinylbenzyl)-bis(2-hydroxyethyl)sulfonium oxalate]                                    | 1.0            | 25.1             | 17.8                          | 3.2              | 13.9                          | 12.7                        |
| 23  | Poly(vinylbenzyl)-bis(2-hydroxyethyl)sulfonium maleate]                                    | 1.0            | 29.9             | 40.4                          | 5.0              | 21.7                          | 16.7                        |
| 24  | Poly(ar-vinylbenzyl)tetrahydrothiophenium chloride]                                        | 1.0            | 37.8             | 69.5                          | 11.3             | 51.1                          | 29.9                        |
| 25  | Poly(ar-vinylbenzyl)(2(2(2(2-hydroxyethoxy)ethoxy)-ethoxy)ethoxy)ethyl sulfonium chloride] | 1.0            | 29.2             | 39.3                          | 5.5              | 25.7                          | 18.5                        |
| 26  | Chloromethylated Polystyrene Treated with Dimethyl Sulfide                                 | 1.0            | 47.8             | 12.7                          | 11.2             | 26.4                          | 23.4                        |

NOTE.—The polymer used in run 26 was prepared by dissolving 10.4 grams of low molecular weight polystyrene (viscosity of 10% soln in toluene at 25° C. equal to 2.0) in 40.3 grams of chloromethyl ether with 0.4 mole of catalyst per aromatic nucleus. After 23 hours at room temp. the reaction was killed in MeOH and the polymer isolated. Chlorine analysis indicated about 80% of the benzene rings had  $-\text{CH}_2\text{C}$  groups attached. 2.24 grams of this polymer was heated at 70° C. with 0.73 gram of dimethyl sulfide and 29.7 ml. of water for about 15 hours. The soluble fraction was tested as indicated above using a kraft pulp.

## EXAMPLE III

Silvace 122, a whole wood (Douglas fir) fiber, was slurried at a 2 percent consistency (based on oven dry weight of fiber) in water.

A solution of poly(vinylbenzyl)bis(2-hydroxyethyl) sulfonium chloride was added and the resulting slurry felted in a conventional deckle box. After dewatering the mat was placed on a screen in a press at 200° C. Pressure was raised to 300 p.s.i. for 1/2 minute and finally to 800 p.s.i. for 4 1/2 minutes. Various concentrations of the sulfonium polymer were used and the resulting boards were tested for the properties and with the results shown in Table XII. The tests were standard ASTM tests (D-1037-52T) modified for size of sample in the case of the water absorption test.

## EFFECT OF POLY(VINYL BENZYL)BIS(2-HYDROXYETHYL)SULFONIUM CHLORIDE OF VARIOUS STRENGTH PROPERTIES OF HARDBOARD MADE BY WET FORMED-WET PRESS PROCESS

| Run | Polymer | Mod. of Rupture, lb./sq. in. <sup>1</sup> | Water Absorption, Percent | Swell Thickness, Percent in $\text{H}_2\text{O}$ | Interanl Bond, lb./sq. in. |
|-----|---------|-------------------------------------------|---------------------------|--------------------------------------------------|----------------------------|
| 1   | 0       | 2,541                                     | 85.0                      | 49.0                                             | 55.0                       |
| 2   | 1/2     | 3,729                                     | 53.1                      | 29.2                                             | 114.0                      |
| 3   | 1       | 4,781                                     | 33.7                      | 23.1                                             | 171.0                      |
| 4   | 1 1/2   | 4,184                                     | 34.0                      | 24.7                                             | 146.0                      |

<sup>1</sup> Corrected to 62.4 lb./cu. ft. density assuming modulus of rupture changes as the sq. of the density.

11  
EXAMPLE IV

Following the procedure of Example III fiber was treated with varying percentages of poly[(vinylbenzyl) dimethylsulfonium chloride], felted, dewatered, oven dried and cured at 107° C. for 3 hours in a forced draft oven to give a 5/8 inch board of about 14 lb./cu. ft. density. The products were tested as in Example III. The results are given in Table XIII.

Table XIII

| Run | Weight Percent Polymer | Modulus of Rupture, lb./sq. in. | Percent Water Absorption |
|-----|------------------------|---------------------------------|--------------------------|
| 1   | 0                      | 22.2                            | 112.4                    |
| 2   | 1/2                    | 28.0                            | 80.0                     |
| 3   | 1                      | 31.5                            | 65.5                     |
| 4   | 2                      | 35.0                            | —                        |

## EXAMPLE V

Ten gallons of "Lady Fair" cleansing tissues and 400 ml. of water or of dilute aqueous solution of poly[dimethyl(ar-vinylbenzyl)sulfonium chloride] microgel (hereinafter designated DMBS microgel) were beaten together for thirty seconds in a Waring blender, the resultant slurries of paper fiber were concentrated on a Buchner funnel to give a soft pulp of about 20% paper solids, and this pulp then pressed through a 3/4 inch glass tube to yield extruded papier-mache samples which were then dried according to two different schedules, the physical appearance noted, and water-resistance determined by placing the samples in beakers of deionized water at room temperature. The results are shown in Table IV. These results show that the control papier-mache samples wetted rapidly and sank within 15 seconds, degenerating to pulpy slush within 15 minutes, whereas the addition of as little as 0.025% of the DMBS microgel to the water slurry produced samples which were firm (requiring a saw to break them) and which remained firm and dry on eight weeks' contact with water.

Table XIV  
EFFECT OF DMBS MICROGEL ON PAPIER-MACHE

| Run | Percent DMBS Microgel <sup>a</sup> in water slurry | Percent Initial water in papier mache | Drying Schedule                                      | Appearance of Dried papier-mache | Water-resistance of papier-mache                                           |
|-----|----------------------------------------------------|---------------------------------------|------------------------------------------------------|----------------------------------|----------------------------------------------------------------------------|
| 1   | None                                               | 61                                    | <sup>b</sup> I<br><sup>c</sup> II                    | weak, crumbly<br>firm            | Wets rapidly; slushy pulp within 15 min.<br>Do.                            |
| 2   | 0.025                                              | 69                                    | <sup>b</sup> I<br><sup>c</sup> II                    | firm, hard<br>do                 | no visible wetting; firm and substantially dry after eight weeks in water. |
| 3   | 0.250                                              | 72                                    | <sup>c</sup> II<br><sup>b</sup> I<br><sup>c</sup> II | do<br>hard, crumbles on sawing   | same as above.<br>same as above.<br>same as above.                         |

<sup>a</sup>Microgel polymer containing 0.05% divinylbenzene.

<sup>b</sup>Schedule I: 16 hrs. at 70° C. and 1 atm., then 24 hrs. at 75° C. under vacuum.

<sup>c</sup>Schedule II: 16 hrs. at 26° C. and 2 mm., then 24 hrs. at 75° C. under vacuum.

This application is a continuation-in-part of our co-pending application Serial No. 6,589, filed February 4, 1960, now abandoned.

What is claimed is:

1. A method for producing cellulosic and lignocellulosic articles which comprises adding from 0.025 to 5.0 weight percent, dry fiber basis of at least one member

5  
10  
15  
20  
25  
30  
35  
40  
45

of the group consisting of (I) homopolymers having the recurring group



wherein R<sub>1</sub> is selected from the group consisting of hydrogen and alkyl radicals containing from 1 to 6 carbon atoms, X is an organic sulfur-containing compound selected from the group consisting of (A) sulfides of the formula R<sub>2</sub>SR<sub>3</sub>, wherein R<sub>2</sub> and R<sub>3</sub> each represents a member of the group consisting of (1) alkyl radicals containing from 1 to 6 carbon atoms, (2) haloalkyl radicals containing from 1 to 6 carbon atoms, (3) hydroxyalkyl radicals containing from 1 to 6 carbon atoms; (4)



where n is an integer from 1 to 4 inclusive; (5)



wherein n is an integer from 1 to 4 inclusive; (6)

—(CH<sub>2</sub>—CH<sub>2</sub>O)<sub>m</sub>CH<sub>2</sub>CH<sub>2</sub>OH wherein m is an integer from 1 to 5; (7) —C<sub>n</sub>H<sub>2n</sub>COOH; (8)

—C<sub>n</sub>H<sub>2n</sub>COOC<sub>n</sub>H<sub>2n+1</sub>; (9) —C<sub>n</sub>H<sub>2n</sub>COO alkali metal; and (10) —C<sub>n</sub>H<sub>2n</sub>CONH<sub>2</sub>; wherein n in substituents (7), (8), (9), and (10) is an integer from 1 to 5 with the total number of carbon atoms in each of the substituents (7), (8), (9), and (10) not exceeding 6, and where the total number of carbon atoms of the R<sub>2</sub> and R<sub>3</sub> groups attached to a common sulfur atom does not exceed 18 and (B) cyclic thio compounds selected from the group consisting of tetrahydrothiophene, hydroxy substituted tetrahydrothiophene, halo substituted tetrahydrothiophene, alkyl substituted tetrahydrothiophene where alkyl refers 45 to groups containing from 1 to 5 carbon atoms, tetrahy-

drothiopyran, and 1-oxa, 4-tetrahydrothiopyran; and Y is an anion from the group consisting of carbonate, oxalate, phthalate, succinate, di-hydrogen phosphate, fluoride, benzoate, chloride, nitrate, acetate, sulfate, bromide, and iodide; (II) copolymer thereof, and (III) copolymers with minor proportions of other ethylenically unsaturated monomers to a slurry of cellulosic and lignocellulosic

**13**

fibers, dewatering the slurry to form an article, and thereafter curing.

2. The method of claim 1 wherein the homopolymer is poly[(vinylbenzyl)bis-(2-hydroxyethyl)sulfonium chloride].

3. The method of claim 1 wherein the homopolymer is poly[(vinylbenzyl)dimethylsulfonium chloride].

4. The method of claim 1 wherein the polymer is a copolymer of poly[(vinylbenzyl)bis-(2-hydroxyethyl)sulfonium chloride] and acrylamide.

5. The method of claim 1 wherein the polymer is a copolymer of poly[(vinylbenzyl)dimethylsulfonium chloride] and styrene.

6. The method of claim 1 wherein the polymer is a copolymer of acrylic acid and poly[(vinylbenzyl)bis-(2-hydroxyethyl)sulfonium chloride].

**14**

7. The method of claim 1 wherein from about 0.1 to 3.0 weight percent of the polymer is added to the fiber slurry.

5        **References Cited in the file of this patent**

UNITED STATES PATENTS

|              |                   |       |               |
|--------------|-------------------|-------|---------------|
| 2,895,925    | Hwa               | ----- | July 21, 1959 |
| 2,923,700    | Price             | ----- | Feb. 2, 1960  |
| 10 2,947,731 | Nummy             | ----- | Aug. 2, 1960  |
| 2,989,520    | Rutenbert et al.  | ----- | June 20, 1961 |
| 3,060,156    | Rassweiler et al. | ----- | Oct. 23, 1962 |

FOREIGN PATENTS

|              |        |       |               |
|--------------|--------|-------|---------------|
| 15 1,031,228 | France | ----- | Mar. 18, 1953 |
|--------------|--------|-------|---------------|

UNITED STATES PATENT OFFICE  
CERTIFICATE OF CORRECTION

Patent No. 3,130,117

April 21, 1964

Charles G. Humiston et al.

It is hereby certified that error appears in the above numbered patent requiring correction and that the said Letters Patent should read as corrected below.

Column 3, line 35, strike out "and", second occurrence; lines 42 and 43, strike out "ethylene glycol, diacrylate,"; column 7, Table VI, second column, line 13 thereof, for "0.01%" read -- 0.1% --; column 8, Table VII, second column, line 1 thereof, for "Newspring" read -- Newsprint --; columns 9 and 10, Table XI, second column, line 10 thereof, for "(carbamoylmetnyl)" read -- (carbamoylmethyl) --; same Table XI, second column, line 30 thereof, for "sulfonium" read -- sulfonium --; column 10, Table XII, sixth column, in the heading thereof, for "Interan1" read -- Internal --; column 12, line 69, for "1-oxa, 4-tetrahydrothiopyran" read -- 1,4-oxathiane --; column 13, lines 9 and 10, for "poly[(vinylbenzyl)bis-(2-hydroxyethyl)sulfonium chloride]" read -- (vinylbenzyl)bis-(2-hydroxyethyl)sulfonium chloride --; lines 12 and 13, for "poly[(vinylbenzyl)dimethylsulfonium chloride]" read -- (vinylbenzyl)dimethylsulfonium chloride --; same column 13, lines 15 and 16, for "poly[(vinylbenzyl)bis-(2-hydroxyethyl)sulfonium chloride]" read -- (vinylbenzyl)bis-(2-hydroxyethyl)sulfonium chloride --.

Signed and sealed this 20th day of October 1964.

(SEAL)

Attest:

ERNEST W. SWIDER  
Attesting Officer

EDWARD J. BRENNER  
Commissioner of Patents